

Patented Jan. 9, 1923.

1,441,243

# UNITED STATES PATENT OFFICE.

ADOLF RÖMER, OF STUTTGART, GERMANY.

## PROCESS FOR OBTAINING TANNING MATERIAL FROM CELLULOSE WASTE SULPHITE LYES.

No Drawing.

Application filed April 9, 1921. Serial No. 480,147.

*To all whom it may concern:*

Be it known that I, ADOLF RÖMER, a German subject, resident of Stuttgart, Germany, have invented certain new and useful Improvements in Processes for Obtaining Tanning Material from Cellulose Waste Sulphite Lyes (for which I have filed applications in Germany, Dec. 24, 1915; Aug. 22, 1917; Jan. 23, 1919; Hungary, June 1, 10 1918, Feb. 11, 1919; Austria, Jan. 27, 1919; France, Aug. 17, 1918; Sweden, Aug. 19, 1919, Jan. 31, 1919; Norway, Feb. 11, 1919), of which the following is a specification.

It has been suggested, for the purpose of 15 obtaining tanning substances from waste sulphite cellulose lyes, to neutralize the lye with lime, and after separation of the calcium sulphite precipitated to mix with metal sulphates such as for instance alum, for the 20 purpose of obtaining tannates of metals with separation of gypsum. Tanning lyes thus obtained, always contain lime which is undesirable for tanning purposes, in the form of tannates of lime, or of gypsum. 25 Another suggestion was to pass sulphite lye neutralized with milk of lime, through an osmotic apparatus, and for the purpose of further conversion into a tanning substance, to free the non-diffusing portion entirely or 30 partly from lime by means of sulphuric acid. But in this case also it is impossible to obtain a solution free from lime. It has been further suggested to free sulphite lyes from lime by means of soda, and to use 35 the solutions which are then preferably mixed with alum, for tanning, but with the addition before, during or after, the tanning process, of diluted acid for the purpose of neutralizing the alkalies released during 40 the tanning which spoiled the colour of the leather on the surface and in section. Such tanning lyes are practically useless as they contain sulphurous acid which is very injurious for tanning. For the purpose of obtaining 45 tanning liquors which are free from lime and sulphurous acid, it has been suggested to free the lye from the chief quantity of sulphurous acid and calcium sulphite by heating or treatment in vacuo, to 50 convert the remaining free and bound sulphurous acid into sulphuric acid by means of ozone, and finally to cause it to react with carbonate of barium.

According to the present process it is possible to obtain in a most simple technical

manner tanning substances with excellent tanning properties, free from injurious ingredients, more particularly from sulphurous acid and lime by converting the acids contained in the waste lyes, such as sulphurous acid, sulpho-lignic acid, etc., or their acid salts, into neutral salts, by means of an alkaline calcium compound such as milk of lime, carbonate of lime or the like, owing to which all sulphurous acid is precipitated in the form of neutral sulphite of lime, whereupon the solution is freed from the substances precipitated, and mixed with suitable alkali compounds, for instance alkali carbonate or alkali silicate, for the purpose of converting the lignine-sulfonates of lime into lignine-sulfonates of an alkali metal, with quantitative precipitation of the lime. The lye thus obtained which contains sulpho-lignic acid in the form of a neutral alkali salt, has no tanning effect; the latter is only obtained when the alkali salt is mixed with a strong acid such as for instance hydrochloric acid or sulphuric acid. It has been found that the quantity of acid 60 added must not be less than half the quantity 65 theoretically required for converting the lignine alkali metal sulfonate into the free sulfonic acid, and not materially more than 70 theoretically required for complete conversion. 75

An advantageous method of carrying out the invention consists in subjecting the lye neutralized with milk of lime or carbonate of lime, after separating the substances thus 80 precipitated, to fermentation. It is preferable in that case to pass the lye through a closed system of fermentation vessels charged with yeast fixed on a carrier. The liquid thus freed from sugar, is then further 85 treated, in the manner already described, with alkali compounds and, after separation of the carbonate of lime precipitated, condensed by evaporation and mixed with acid. By fermenting the sugar, not only alcohol is 90 obtained, but the tanning extract is improved by the removal of the sugar which is 95 a non-tanning substance.

Another modification of the invention consists in acting on the lignine-sulfonates of 100 alkali metals not with hydrochloric acid or sulphuric acid, but in using in their place acid-reacting salts of metals such as are utilized for the purpose of mineral tanning, for instance aluminium chloride, ferric chlo- 105 110

ride or chromium-chloride. Compound tanning substances with specially favourable properties are thus obtained. They quickly and completely penetrate into the animal 5 hide both in concentrated and in diluted solution, so that in both cases excellent and fully tanned leather is obtained.

A specially remarkable behaviour is that of ferric oxide salt. As is well known, in 10 iron tanning the effective ferric oxide salts cannot be used directly for tanning, as they do not penetrate into the hide. In order to ensure tanning right through it was hitherto necessary to treat the unhaired skins with 15 non-tanning ferrous oxide salts which have a better diffusion property, and to convert them on the hide into tanning ferric oxide salts by oxidation. It is therefore surprising that ferric oxide salt of sulfo-lignic 20 acid can be successfully used directly for tanning.

Example. The waste sulphite lye is supersaturated with milk of lime or with chalk. Other disturbing impurities, more particularly resin-like substances, are precipitated 25 at the same time. The remaining solution is thereupon treated with sodium carbonate, and to the liquid separated from the precipitate, is added half of the amount of hydrochloric acid or of one of the above mentioned 30 metal chlorides, theoretically required for binding the alkali metal of the alkali metal lignine-sulfonates. The amount of acid or of the acid-reacting metal salt can be determined 35 in a very simple manner, as the quantity of soda consumed for the conversion of lignine-sulfonate compound of lime, gives directly the measure of the acid addition. By evaporating the solutions prepared in 40 accordance with the present process, highly efficient tanning extracts are obtained, which in addition to the already mentioned advantages of the absence of injurious and undesired substances, have also the great advantage 45 of always being of uniform efficacy, a very important property for properly regulating tanyard working, which is absent in most extracts obtained from sulphite lyes. A special advantage is that formation of 50 free mineral acids is avoided in any case.

Having now particularly described and ascertained the nature of my said invention and in what manner the same is to be performed, I hereby declare that what I claim 55 is:—

1. A process for obtaining tanning substances from waste sulfite cellulose lye consisting in first subjecting the lye to the action of an alkaline calcium compound for 60 the purpose of precipitating all of the sulfurous acid, then removing the precipitate and subjecting the remaining solution to the action of alkali compounds capable of precipitating the calcium combined with the sulfo-lignic acids 65 thereby converting the lignine compounds into alkali metal lignine sulfonates and lastly treating said alkali metal lignine sul-

lignine compounds into alkali metal lignine sulfonates and lastly treating said alkali metal lignine sulfonates with a compound of acid character.

2. A process for obtaining tanning substances from waste sulfite cellulose lye consisting in first subjecting the lye to the action of an alkaline calcium compound for the purpose of precipitating all of the sulfurous acid, then removing the precipitate 70 and subjecting the remaining solution to the action of alkali compounds capable of precipitating the calcium combined with the sulfo-lignic acids thereby converting the lignine compounds into alkali metal lignine 75 sulfonates and lastly treating said alkali metal lignine sulfonates with a compound of acid character whereby the quantity of the latter is less than the quantity required for combining with all of the alkali metal 80 of the lignine-sulfonate.

3. A process for obtaining tanning substances from waste sulfite cellulose lye consisting in first subjecting the lye to the action of an alkaline calcium compound for 90 the purpose of precipitating all of the sulfurous acid, then removing the precipitate and subjecting the remaining solution to the action of alkali compounds capable of precipitating the calcium combined with the sulfo-lignic acids thereby converting the lignine compounds into alkali metal lignine sulfonates and lastly treating said alkali metal lignine sulfonates with a compound 95 of acid character whereby the quantity of the latter is about one half of the quantity required for combining with all of the alkali metal 100 of the lignine-sulfonate.

4. A process for obtaining tanning substances from waste sulfite cellulose lye consisting in first subjecting the lye to the action of an alkali calcium compound for the purpose of precipitating all of the sulfurous acid, then removing the precipitate 105 and subjecting the remaining solution to fermentation, then treating it with alkali compounds capable of precipitating the calcium combined with the sulfo-lignic acids thereby converting the lignine compounds into alkali metal lignine sulfonates and lastly treating 110 said alkali metal lignine sulfonates with a compound of acid character.

5. A process for obtaining tanning substances from waste sulfite cellulose lye consisting in first subjecting the lye to the 115 action of an alkaline calcium compound for the purpose of precipitating all of the sulfurous acid, then removing the precipitate and subjecting the remaining solution to fermentation, then treating it with alkali compounds capable of precipitating the calcium combined with the sulfo-lignic acids thereby converting the lignine compounds into alkali metal lignine sulfonates and lastly treating said alkali metal lignine sul-

- fonates with a salt of a metal suitable for mineral tanning.
6. A process for obtaining tanning substances from waste sulfite cellulose lye consisting in first subjecting the lye to the action of an alkaline calcium compound for the purpose of precipitating all of the sulfurous acid, then removing the precipitate and subjecting the remaining solution to 5 fermentation, then treating it with alkali compounds capable of precipitating the calcium combined with the sulfo-lignic acids thereby converting the lignine compounds into alkali metal lignine sulfonates and 10 lastly treating said alkali metal lignine sulfonates with a salt of a metal suitable for mineral tanning in a quantity insufficient to convert all of the alkali metal lignine sulfonate into the metal lignine sulfonate.
7. A process for obtaining a tanning substance from waste sulfite liquor consisting in first adding to the liquor calcium carbonate to precipitate all of the sulfurous acid, then removing the precipitate and subjecting the remaining solution to the action of alkali metal carbonate, thereby converting the lignine compounds into alkali metal lignine-sulfonates and then adding hydrochloric acid in a quantity insufficient to combine with all of the alkali metal of the lignine sulfonate.

In testimony whereof I have signed my name to this specification in the presence of two subscribing witnesses.

DR. ADOLF RÖMER.

Witnesses:

WILHELM STÄHLE,  
AUGUST FREY.